

April 20, 1926.

1,581,790

J. C. DAVIS

CASTING AND METHOD OF PRODUCING THE SAME

Filed Nov. 13, 1922 2 Sheets-Sheet 1

Fig. 1



Fig. 2



Fig. 3



Witness:-

Inventor  
James Carey Davis  
By Lane Carpenter

April 20, 1926.

1,581,790

J. C. DAVIS

CASTING AND METHOD OF PRODUCING THE SAME

Filed Nov. 13, 1922

2 Sheets-Sheet 2

Fig. 4



Fig. 5



Witness:  
Harry A. Hitzman

Inventor  
James C. Davis  
By  
John Carpenter  
Atty.

Patented Apr. 20, 1926.

1,581,790

# UNITED STATES PATENT OFFICE.

JAMES CAREY DAVIS, OF HINSDALE, ILLINOIS.

## CASTING AND METHOD OF PRODUCING THE SAME.

Application filed November 13, 1922. Serial No. 600,656.

*To all whom it may concern:*

Be it known that I, JAMES CAREY DAVIS, a citizen of the United States, and a resident of Hinsdale, in the county of Du Page and State of Illinois, have invented certain new and useful Improvements in Castings and Methods of Producing the Same, of which the following is a specification.

My present invention relates to the art 10 of casting metal, and to improve means and methods for producing castings which are not only smooth and "clean" in that they are free from pits or holes and from entrained dirt such as sand, but are notably dense as 15 well as solid.

Pits, holes, dirt, and the like involve roughness, flaking, shelling, and a consequent cutting action, since they cannot readily be machined out, and other obvious 20 imperfections with an incident intolerably great manufacturing cost due to the high scrap loss of the castings necessarily discarded on account of inavailability for the purposes contemplated.

It will be appreciated that castings of 25 high quality, the attainment of which is one of my present objectives, are useful for many purposes, but are not only of utility but practically essential for a number of 30 uses, such for example as car-wheels and other structures more or less analogous in certain characteristics.

The case of car-wheels is an example for 35 which the invention is peculiarly adaptable, inasmuch as where desirable, additionally a hardening or other modifying element may be so introduced at such a place and stage and so regulated and determined, and with such degree of nicety as may be desired, 40 that not only a solidity but also homogeneity of metal throughout the casting, or certain parts thereof, may be secured but also that the repeated production of a run of castings of like composition and density may be attained.

The castings produced by my present improvements may be of uniform composition throughout, or the introduction of a modifying element referred to may be effected 50 when, if and as desired, thus in the furnace or cupola, in the ladle, or between the ladle and the mold, whereby the casting may be of differing composition in different parts.

For the purpose of illustration of the present invention in its various aspects, I have 55 therefore found it convenient in the present

specification and drawings to refer to it in connection with its adaptability for car-wheels and the like, which may be of uniform or variable composition, according to 60 the service in view.

In the production of such castings by other means and methods known to me I have heretofore experienced great difficulty not only in accurately apportioning the 65 modifying element when desired but in attaining the requisite solidity and density in the castings and in insuring a constant run of castings which are both of the composition, solidity and density sought for, but at 70 the same time free from insuperable peripheral imperfections such as foreign matter, shelling, irregularities of contour, etc., which are intrinsic and more than merely superficial and so involve actual rejection 75 of the product.

The principal objects of my present invention therefore involve the provision of an improved casting apparatus adapted for the inclusion of means for the production 80 of castings of quite perfect solidity and great density; the provision of such an apparatus characterized by the inclusion of means whereby such density may be intensified at predetermined localities; the provision of such an apparatus adapted for the production of castings of varying density, or varying both in density and composition; the provision of a casting apparatus characterized by the employment of an 85 auxiliary source of molten metal for imparting solidity and high density to the casting; the provision of a casting apparatus including a rotating mold for such purpose; the provision of an improved mold having 90 means for receiving an ancillary source of molten metal, one wherein such ancillary source may be drawn upon to compensate for shrinkage in the casting as it cools or entrained gases are expelled from the casting 95 or from the mold, and one adapted to facilitate the escape of gas from the mold cavity; the production of a casting further characterized by predetermined variation in its density; the provision of such a casting 100 further characterized by predetermined variation in its composition; and generally the provision of a greatly improved form of casting having novel inherent structural and qualitative features and properties, and one 105 which differs in kind as well as degree from those hitherto known.

100

105

110

The principal objects of my present invention further contemplate the utilization of an improved method of making castings, which are of varying density in different portions, and, when if and as desired of differing degrees of hardness in different portions, together with certain other objects which will be hereinafter disclosed.

In the attainment of the objects and advantages above noted, in the avoidance of the objections and disadvantages mentioned, and in accomplishing certain ends and gaining certain benefits which will below be pointed out or clearly appear, I have provided the constructions illustrated in the accompanying drawings which for purposes of convenience as before suggested are adapted for the production of a car-wheel such as one made of steel which is solid, dense, hard and resistant and consequently of excellent wearing qualities at the peripheral or tread portion, and may be relatively softer toward the center and therefore more tough and less apt to fracture.

In these drawings, it will be observed that in—

Figure 1 I have illustrated a mold provided with means for rotating the same, and a ladle for introducing molten metal into the mold, the mold being provided with ancillary means for supplying additional molten metal to the casting proper as it shrinks, the mold and casting being shown in central longitudinal section;

Figure 2 a plan view of the mold of Figure 1;

Figure 3 a view of the casting therein produced;

Figure 4 an elevational view of a modified form of apparatus; and in

Figure 5 a plan view of part of the apparatus of Figure 4.

Referring first to the apparatus of Figures 1, 2 and 3, it will be noted that I may employ a mold, such as the car wheel mold 6, which is preferably mounted upon a support 7 which is rotatable by means of a suitable driving mechanism indicated generally at 8. The mold 6 is provided with a pouring gate 9 having a refractory lining 10 for directing into the mold molten metal from the ladle 11 or the like.

Interiorly the mold 6 is provided with an ancillary receptacle for molten metal, the excess of which will not form part of the finished casting. In the case of the production of such a casting as the car-wheel shown in Figure 3, I conveniently employ two such receptacles which take the form of sinking heads 12, 12 in the cope 13 of the mold 6. In the resultant castings such remainder of the redundant metal from the sinking heads 12, 12, indicated at 12<sup>a</sup>, 12<sup>a</sup>, are of course duly removed, before they are put into use.

Referring now to the apparatus of Figures 4 and 5, it will be seen that I here mount in a convenient place as in a pit, the desired number of molds 6, each of which is mounted on a rotatable table 7 driven by gearing 8.

For the purpose of providing means whereby the molten metal from the ladle 11 may be maintained at a height substantially uniform and will thereby be caused to descend in a solid column of uniform diameter, contour and velocity, I provide a choke device comprising a hopper or funnel 19, preferably conically shaped, the open bottom of which is partially closed by a nozzle 20 which is formed of refractory material and may be renewed from time to time as required in service. To the end that the choke device may be centered over the pouring gate 17, and where circumstances render it desirable moved from one flask to another, it is mounted upon a truck 21 which comprises a supporting bed 22 carried upon axles 24 the wheels of which are revoluble thereupon and arranged to ride upon rails 26 the outer ends of which are mounted upon trucks 27 and 28 which in turn ride upon the rails 29 and 30 oppositely disposed about the molds 6.

In carrying out my improved process of making castings, the modifying element, such as manganese may be added in the furnace or cupola, or in the ladle 11, or between the ladle 11 and the mold 6, but for the purpose of introducing and incorporating most perfectly and commingling and distributing most thoroughly the modifying element into the stream of flowing metal 31, which as will be seen on reference to Figure 4 preferably takes the form substantially of a column with parallel sides, I may make use of an apparatus which here comprises a vertical casing 32 for containing the modifying elements, such as manganese, a lateral extension thereof 33, a nozzle 34 the ejector of which, 35 is depressed somewhat from the horizontal, and a pipe 36 connected to a source of air or other fluid pressure supply, and inserted into the apparatus below the casing 32 to the end that the modifying element may be drawn therefrom by fluid pressure and forced into the flowing stream of metal. In practice, I have found that the best results are attained by the use of pressures between approximately 50 and 125 lbs. per square inch which will cause the modifying element to penetrate the stream of molten metal, and that by flattening the ejector 35 so that the spray of modifying material may be spread out to approximately the diameter of the stream, and depressing the end of the ejector so that the modifying material will strike the flowing stream in the direction in which it flows, it will enter and be more thoroughly commingled and homogene-

ously incorporated with the molten metal, and will not have the tendency to become segregated in masses therein nor to be unevenly disposed therein, nor to remain on the surface of the stream and subject to the action of the air.

For certain purposes it is highly desirable to attain an accurate and uniform proportioning of the quantities of the modifying

10 element and molten metal as they enter the mold. In order to do this, obviously it is not only desirable to have the modifying element delivered in uniform and unvarying quantity, but it is also desirable to have the 15 molten metal delivered in uniform and unvarying quantity. If the metal be taken di-

rectly from a pouring ladle of the ordinary type its velocity will vary as the height of the metal in the ladle varies. From this it

20 follows that if the rate of flow of the modifying element be uniform, the proportion of the modifying element and metal delivered to the mold will vary, because the rate of flow of the metal is not uniform. In

25 overcoming this I have provided a choke device whereby I am enabled to maintain the height of the metal in that device substantially uniform. As a result, the discharge of metal into the mold is uniform.

30 Furthermore, as the head of metal in the choke device is relatively small, the issuing stream is in the form of a substantially solid column. Furthermore, by employing the injecting device referred to, the modifying element is immediately embedded in and firmly held by the flowing metal, and is 35 therefore uniformly carried into the mold.

In the production of a wheel of uniform composition I preferably employ molten 40 steel having a specification of 0.25 to 0.50% carbon and 1.25 to 2.0% manganese, which may be introduced in the furnace, though it

45 will be understood my present improvements are available for the production of wheels having a varying composition by graduating the addition of the modifying material as can be accomplished readily by introducing it between the ladle and the mold for example.

50 The molten metal is then poured into the mold 6 and as such mold fills the ancillary mold cavities are filled and the sinking heads 12, 12 are formed.

55 The pouring being finished, rotation of the mold is effected until the casting is solidified, when it is removed from the mold and the excrescences 12<sup>a</sup>, 12<sup>a</sup> are removed and the customary finishing operations are performed.

60 From experience I have ascertained that if the mold 6 remains stationary I cannot infallibly attain the degree of solidity and density in the castings, desired by me, but that by utilizing a rotating mold at say 25 to 65 100 R. P. M. centrifugal motion is im-

parted to the molten metal to such an extent that the metal filling the sinking heads 12, 12 serves to completely fill the outermost parts of the mold 6 in such a manner that I am not only enabled to prevent the formation of holes and secure a solid and clean casting, but am enabled to attain in addition to highly complete solidity a marked degree of density.

Inasmuch as I preferably make use of 75 centrifugal force the extent to which the benefit thereof is attained obviously depends in part upon the rate of revolution imparted to the mold 6 and in part the time interval through which such movement is continued.

It is believed that the operation of my present invention and various applications of its use will be understood by those skilled in the art without further detailed description.

85 For certain purposes and in certain of its phases it may be employed in connection with stationary molds, in intermittently rotated molds, in continuously rotated molds, and in molds rotated at predetermined times, and equally the modifying material may be introduced at various points or under various conditions, or both, all according to the prospective uses of the castings 90 produced.

95 In the claims where I use the terms "to preferentially densify", "to preferentially compensate", "to preferentially solidify", or "to preferentially condense", I mean to include such property as would be obtained in rotary casting wherein an ancillary supply of molten metal is included as would favor the addition of molten metal from the ancillary supply to the periphery of the casting 100 rather than to the body of the casting.

Having thus described my invention and illustrated its use what I claim as new and desire to secure by Letters Patent is:

110 1. The method of casting car wheels which includes introducing molten metal into a mold and then rotating the mold after pouring so as to impart centrifugal motion to the molten metal to force it outwardly to the confines of the mold to an extent sufficient to densify the metal of the periphery of the casting.

115 2. The method of making car wheel castings which includes pouring molten metal into a mold including an ancillary chamber closed to the atmosphere and introducing metal in said chamber to provide an ancillary supply of molten metal to preferentially compensate for rim shrinkage of the first mentioned metal as it cools.

120 3. The method of making car-wheel castings which includes incorporating through a main pouring gate molten metal into a mold also including an ancillary metal retaining means and introducing molten metal

in said means to furnish an ancillary supply of metal and rotating the mold to impart centrifugal motion of the first mentioned molten metal and thereby draw into the mold a supply of the last mentioned molten metal to an extent sufficient to preferentially densify the metal of the periphery of the casting.

4. The method of making car-wheel castings which includes incorporating molten metal into a mold including an ancillary metal retaining means and introducing molten metal in said means to furnish an ancillary supply of metal and rotating the mold as to impart centrifugal motion to the first mentioned molten metal, and thereby draw into the mold a supply of the last mentioned molten metal to an extent sufficient to preferentially solidify the metal of the periphery of the casting.

5. The method of making castings which includes incorporating molten metal into a mold including an ancillary metal retaining means and introducing molten metal in said means to furnish an ancillary supply of metal and rotating the mold to impart centrifugal motion to the first mentioned molten metal and thereby draw into the mold a supply of the last mentioned molten metal to an extent sufficient to preferentially solidify the metal of the casting with a force characteristic of the centrifugal force of substantially rim velocity.

6. The method of making castings which includes incorporating molten metal into a mold including an ancillary metal retaining means and introducing molten metal in said means to furnish ancillary supply of metal and rotating the mold as to impart centrifugal motion to the first mentioned molten metal, and thereby draw into the mold a supply of the last mentioned molten metal to an extent sufficient to preferentially condense and solidify the metal of the casting with a force characteristic of the centrifugal force of substantially rim velocity.

7. The method of making car-wheel castings which includes introducing molten metal into a mold and an ancillary metal retaining means to provide an ancillary supply of molten metal, and rotating the mold after it is poured so as to impart centrifugal motion to the first mentioned molten metal, and thereby draw into the mold a supply of the last-mentioned molten metal.

8. The method of making castings which includes pouring into a mold a mixture of fluid metal and a modifying element and rotating the mold after it is poured.

9. The method of making car-wheel castings which includes pouring into a mold a mixture of fluid metal and a modifying element and rotating the mold after it is poured at a rate of speed sufficient to condense the outer portions of the metal.

10. The method of making car-wheel castings which includes pouring into a mold a mixture of fluid metal and a modifying element, the modifying element being forced into the stream of molten metal in substantially the same direction as the flow thereof between the ladle and the mold, and rotating the mold after it is poured.

11. The method of making car-wheel castings of varying composition and density which includes introducing into a mold a stream of metal in the form of substantially a solid column, forcing a graduated supply of a modifying element into the column between the ladle and the mold, said mold being provided with an ancillary metal retaining means adapted to provide an ancillary supply of metal, and rotating the mold after the casting is poured to force metal into the mold from the ancillary supply.

12. In a casting apparatus, in combination with a source of molten metal, and a mold, and means for rotating the same, a limited ancillary source of molten metal for preferentially compensating for shrinkage in the casting after the pour from said first mentioned source is completed and as the mold is rotated.

13. In a rotary casting apparatus, a mold provided with a pouring gate, and ancillary means closed to atmosphere for receiving molten metal from the main body of metal for the formation of a casting therein.

14. In a rotary casting apparatus, a mold provided with a pouring gate, and an ancillary sinking head closed to atmosphere for receiving molten metal for the formation of a casting therein.

15. In a rotary casting apparatus, a car wheel mold provided with a pouring gate, and internal ancillary means for receiving molten metal for the formation of a casting therein disposed near the periphery of the wheel.

16. In a rotary casting apparatus, a car wheel mold provided with a pouring gate, and an interiorly disposed ancillary sinking head closed to atmosphere for receiving molten metal for the formation of a casting therein disposed near the periphery of the wheel.

17. As a new article of manufacture, a car wheel casting of predetermined uniform progressive variation in density at different points as produced by substantially completely pouring in a mold and then rotating the same.

18. As a new article of manufacture, a car wheel casting of predetermined uniform progressive variation in density at different points decreasing from the periphery inwardly as produced by substantially completely pouring in a mold and then rotating the same.

19. As a new article of manufacture, a

car wheel casting peripherally condensed by centrifugal force during the course of manufacture when the metal is fluid and the casting has been poured as produced in a rotary mold including an internal ancillary supply of molten metal intermediate the axis and the periphery of the casting.

20. As a new article of manufacture, a car wheel casting containing 0.25 to 0.50% carbon and condensed during the course of manufacture when the metal is fluid and the casting has been poured as produced in a rotary mold including an internal ancillary supply of molten metal intermediate the axis and the periphery of the casting.

21. As a new article of manufacture, a car wheel casting containing 1.25 to 2.0% manganese and condensed during the course of manufacture when the metal is fluid and the casting has been poured as produced in a rotary mold including an internal ancillary supply of molten metal intermediate the axis and the periphery of the casting.

22. As a new article of manufacture, a car wheel casting containing 0.25 to 0.50% carbon, and 1.25 to 2.0% manganese and peripherally condensed during the course of manufacture when the metal is fluid and the casting has been poured as produced in a rotary mold including an internal ancillary supply of molten metal intermediate the axis and the periphery of the casting.

23. A new article of manufacture, a car wheel casting containing 0.25 to 0.50% carbon, and 1.25 to 2.0% manganese and condensed during the course of manufacture by rotation of the mold when the metal is fluid and the casting has been poured as produced in a rotary mold including an internal ancillary supply of molten metal intermediate the axis and the periphery of the casting.

24. The method of making car wheel castings which includes pouring into a mold a mixture of fluid metal and a modifying element, the modifying element being introduced between the ladle and the mold, in substantially the direction of the flow of the stream of molten metal, and rotating the mold after it is poured.

25. The method of making car wheel castings which includes pouring into a mold a mixture of fluid metal and a modifying element, the modifying element being forced into the stream of molten metal in substantially the same direction as the flow thereof between the ladle and the mold, and rotating the mold after it is poured.

26. The method of manufacturing a car wheel casting, which comprises introducing molten metal into a mold; including an internal ancillary means of retaining the molten metal located near the periphery of the casting and then rotating the mold for con-

densing the molten metal at the outer portion of the casting.

27. The method of manufacturing a casting, which comprises introducing molten metal together with a modifying substance into a mold including an internal ancillary means for retaining molten metal located near the periphery of the casting and then rotating the mold for condensing the molten metal at the outer portion of the casting.

28. In a device of the character described, in combination, a source of molten metal, a mold and means for rotating same, and an ancillary limited source of molten metal located between the axis and the periphery of the casting intermediate the confines thereof.

29. In a casting apparatus, in combination with a source of molten metal, and a mold, and means for rotating the same, and ancillary limited source of molten metal located between the axis and periphery of the casting intermediate the confines thereof for compensating for shrinkage in the casting after the pour from said first mentioned source is completed.

30. The method of making castings which includes introducing molten metal into a mold including an ancillary metal retaining means, rotating the casting to impart centrifugal force against the periphery of the casting and augmenting the supply of metal in direction of the centrifugal motion with a force characteristic of the centrifugal force at points within the limits of the body of the rotating casting.

31. The method of making car wheel castings which includes introducing molten metal in a mold including an ancillary metal retaining means, rotating the casting to impart centrifugal force against the periphery of the casting and augmenting the supply of metal from the said ancillary means, intermediate the axis and periphery of the casting at substantially the tread momentum.

32. In the process of molding castings in a rotating mold, the step which includes introducing an ancillary supply of molten metal near the peripheral portion intermediate the axis and the body of the casting.

33. In the process of molding castings in a rotating mold, the steps which comprise introducing metal into the mold and forcing in an ancillary supply of metal under pressure at points intermediate the axis and the periphery of the body of the casting.

34. In the process of molding castings in a rotating mold, the steps which comprise introducing metal into the mold and forcing in an ancillary supply of metal under pressure substantially equal to that induced by the peripheral momentum of the rotating casting.

JAMES CAREY DAVIS.